

## UNITED STATES PATENT OFFICE

2,642,366

METHOD OF COATING SHEET MATERIAL  
WITH WAXGeorge G. Rumberger, Neenah, Wis., assignor to  
Marathon Corporation, Rothschild, Wis., a cor-  
poration of WisconsinNo Drawing. Application March 23, 1951,  
Serial No. 217,299

17 Claims. (Cl. 117—103)

1

This invention relates to a method of coating sheet materials with hot melt coatings. More specifically this invention relates to an improvement in the method of coating sheet materials, such as paper, paperboard, regenerated cellulose, rubber hydrochloride, polyethylene and other plastic films and the like, with hot melt surface coatings wherein the coatings are cooled under controlled conditions to prevent the formation of irregular flow lines therein, sometimes known in the art as "crow's feet," whereby the production of smooth, uniform and even surface coatings is insured. This application is a continuation in part of my application Serial No. 784,929 filed November 8, 1947, now abandoned.

In the application of water-proof or water-vapor-proof coating materials, such as wax, wax compositions and wax-like resinous coatings to sheet materials by the hot melt method, it is the practice to apply the coating composition in a molten state, and then to chill the coating rapidly in order to set the composition before it has completely penetrated the sheet material, so as to form a superficial surface coating. The cooling operation is generally conducted either by passing the coated sheet material over refrigerated rolls or by contacting the coated sheet material with cold water, such as passing it through a cold water bath. When the latter method of cooling is employed, increased rates of cooling are possible due to the fact that the cooling liquid comes into intimate contact with the surface film. Substantially the same practice is followed in coating pre-cut paperboard carton blanks where it is the practice first to apply the coating material, remove the excess, and rapidly plunge the coated blank into cold water to set the coating. Processes of coating wherein the coating material is cooled by immersion in water are called "water-waxing."

It has been found, however, that when water is employed as a cooling medium for the immersion of the coated sheet material, as in standard commercial production, irregular flow lines, crevices, ridges and other irregularities referred to as crow's feet appear on the surface film. Due to these irregularities in the surface the coated sheets are less glossy than similar coated sheets having a smooth coating. Furthermore, there is a distinct tendency for a coating having these irregularities in the surface to scuff or rub off.

After considerable experimentation with the factors involved in the hot melt coating of wax compositions, specifically in water-waxing, I found that crow's feet are produced on the sur-

2

face of hot melt coatings by turbulence in the cooling water. Under ordinary commercial conditions this turbulence is caused by the agitation of the cooling bath by the sheet material traveling therethrough at the high speeds required in commercial production of coated sheets, or in the case of carton blanks by both the high speed and the intermittent flow of material. Following this discovery I have developed a method whereby microscopic crow's feet or flow lines can be reduced or eliminated under commercial operating conditions even at high speeds of operation, such as at about 300 feet per minute and above, and particularly at speeds in the range of about 500 to about 1000 feet per minute, by adjusting the surface tension of the cooling liquid so that it approaches the surface tension of the applied coating. Crow's feet are thereby minimized or completely eliminated even though the cooling liquid is in a state of turbulence, whether resulting from high speeds of operation or created by other means. The elimination of flow lines in the coating improves the gloss and also the resistance of the coating to rub off or scuff.

Hydrocarbon waxes, such as paraffin wax, which are used in coating sheet materials have in general a surface tension of from about 25 to about 29 dynes per centimeter (d./cm.) when measured at 180° F. At higher temperatures these values would be somewhat lower. When waxes are compounded with other materials for use as moisture-proof and water-vapor-proof coatings, the surface tension of the resulting composition may be greater or less than these values, and the surface tension of the cooling liquid should be adjusted accordingly. I have found that, in general, coating compositions suitable for this purpose have surface tensions at the temperature of application in the range of about 20 to about 40 d./cm. In general, the temperature range at which these coatings are applied will be from about 130° F. to about 300° F. The difference between the temperature of application and the temperature at which the coating contacts the bath will not be sufficient to make any substantial change in the surface tension. As examples of such compositions, I may add to the paraffin wax, alone or in combination, such materials as polyethylene, polyisobutylene, ester gum, microcrystalline wax, metallic soaps, rubber, amides, such as stearamide or stearanalid, antioxidants, such as butylated hydroxy anisole or other phenols, or other materials required to modify the wax to make it suitable for the need at hand, which may modify the surface tension

of the composition. The hydrocarbon wax portion of the composition will, in general, be more than 50% by weight. The viscosities of these compositions at their application temperature will vary with the composition, but they do not generally exceed about 100 centistokes at such temperature. I have found no necessity for having the surface tension of the coolant below that of water when higher viscosity compositions are applied or, in other words, I have found that flow lines or crow's feet do not occur during water-waxing with compositions having a viscosity in excess of about 100 centistokes at the application temperature.

For very high speed coating, or when turbulence is high in the cooling bath for other reasons, I have found that the best results are obtained if the surface tension of the cooling liquid at its temperature exceeds that of the coating composition at the temperature it contacts the coolant by not more than about 5 d./cm. For relatively lower speeds of operation the surface tension of the coolant preferably should not exceed that of the coating composition by more than about 20 d./cm. although in cases where the viscosity of the coating is more than about 50 centistokes at the temperature of contact this difference may be even greater. In general, any lowering of the surface tension below that of water will benefit the coating to some degree. However, for the class of compositions to which my invention is applicable, I have found that the surface tension of the coolant should in no case exceed about 60 d./cm. at its operating temperature, and for hydrocarbon wax and modified wax compositions having a viscosity of less than about 50 centistokes at the temperature of contact, the upper limit is preferably about 45 d./cm. I have found that if the surface tension of the coolant is in the range of about 3 to about 20 d./cm. above that of the coating at their respective temperatures during coating, which may be 50° F. and 180° F. respectively, good results are obtained.

In some cases a coolant having a surface tension equal to or lower than the coating composition may be used. In these cases, however, the coolant wets the coating composition to such an extent that the coolant is subsequently difficult to remove. When these coolants are used, or where complete removal of the coolant is desired, I prefer to chill the sheet sufficiently to congeal the coating, then pass the sheet through a washing bath of water, or other liquid of higher surface tension and having a high solvency for the first coolant, then remove the washing liquid. For example, when cooling a coating composition having a surface tension of about 28 d./cm. in a coolant having a surface tension of about 25 d./cm., I remove as much

coolant as possible by physical means, such as scrapers, rollers, or suction tubes, then pass the sheet through a washing bath of cold water to remove the residual coolant, then remove the water by physical means.

It is obvious that coolants having an appreciable solvency for, or deleterious action on, the composition cannot be used. Therefore, I prefer to use aqueous or alcoholic cooling solutions. For reasons of economy aqueous coolants containing alcohols are preferred. Furthermore, aqueous solutions are less toxic and hazardous to handle.

The following Table I gives results obtained when 24-pounds per ream (24x36—480) opaque sulfite breadwrapper stock was waxed with 130/32° F. ASTM melting point paraffin wax having a surface tension of 28 d./cm. at 180° F., the temperature of application, and cooled by immersing in various cooling liquids which were agitated by blowing a stream of air into the cooling bath with sufficient pressure to cause turbulence.

Table I

| Example | Composition of Cooling Bath                                 | Surface Tension of Cooling Bath, d./cm. at 50° F. | Crow's-Feet Produced |
|---------|-------------------------------------------------------------|---------------------------------------------------|----------------------|
| 1       | 100% Water                                                  | 72                                                | Pronounced.          |
| 2       | 20% Isopropyl alcohol; 80% Water.                           | 35                                                | Very slight.         |
| 3       | 30% Ethyl alcohol; 70% Water.                               | 33                                                | Do.                  |
| 4       | Water Saturated with Heptanol at 40° F.                     | 36                                                | Do.                  |
| 5       | 1.8% Iso amyl alcohol; 0.2% Isopropyl alcohol; 98.0% Water. | 37                                                | Do.                  |
| 6       | 2.7% Iso amyl alcohol; 0.3% Isopropyl alcohol; 97.0% Water. | 36                                                | None.                |
| 7       | 0.1% Di octyl sodium sulfosuccinate; 99.9% Water.           | 26                                                | Do.                  |
| 8       | 0.025% Di octyl sodium sulfosuccinate; 99.975% Water.       | 30                                                | Do.                  |
| 9       | 0.0125% Di octyl sodium sulfosuccinate; 99.9875% Water.     | 40-45                                             | Very slight.         |
| 10      | 0.5% Alkyl Aryl sodium sulfonate; 99.5% Water.              | 32                                                | None.                |

The following Table II gives data obtained in 50 experiments conducted on a high speed water-waxer when 24-pounds per ream (24x36—480) opaque sulfite breadwrapper stock was water-waxed at various speeds, using paraffin wax with a surface tension of approximately 27 d./cm. at 180° F., the temperature of application, and cooling in water having a surface tension of 72 d./cm. at the indicated temperature. Similarly, the waxed sheets were immersed in a solution of isopropyl alcohol in water having a surface tension of 31 d./cm.

Table II

| Example | Waxing Conditions |               |                                              | Properties of Waxed Paper |        |             |
|---------|-------------------|---------------|----------------------------------------------|---------------------------|--------|-------------|
|         | Speed, Ft./min.   | Coolant       | Surface Tension of Coolant, d./cm. at 45° F. | Gloss, Percent            | Scuff  | Crow's-Feet |
| 11      | 630               | Water         | 72                                           | 55                        | Great  | Pronounced. |
| 12      | 630               | Alcohol-Water | 31                                           | 62                        | Slight | None.       |
| 13      | 855               | Water         | 72                                           | 55                        | Great  | Pronounced. |
| 14      | 855               | Alcohol-Water | 31                                           | 61                        | Slight | None.       |
| 15      | 930               | Water         | 72                                           | 54                        | Great  | Pronounced. |
| 16      | 930               | Alcohol-Water | 31                                           | 57                        | Slight | None.       |

From Table II it is seen that by lowering the surface tension to 4 d./cm. above the surface tension of the coating crow's feet were eliminated over a wide range of commercial production speeds. In each case where crow's feet was eliminated, gloss and scuff were materially improved.

The following examples in Table III show the effect of using low surface tension coolants to cool several wax compositions having a viscosity of less than 100 centistokes at 210° F. comprising polyethylene (P. E.) of 7000 molecular weight, paraffin wax and microcrystalline (micro) wax when coated at a temperature of about 175° F. on commercial equipment at high speeds.

Table III

| Ex. | Composition                                                                                            | Speed, Ft./Min. | Surface Tension of Coolant, d./cm. at 50° F. | Surface Tension of Composition, d./cm. at 175° F. | Crow's-Feet | Gloss, Percent |
|-----|--------------------------------------------------------------------------------------------------------|-----------------|----------------------------------------------|---------------------------------------------------|-------------|----------------|
| 17  | 5% polyethylene; 25% 145/47° F. microwax; 70% 130/32° F. paraffin wax.                                 | 700             | 70                                           | 28-29                                             | heavy...    | 67             |
| 18  | Same as 17                                                                                             | 780             | 40                                           | 28-29                                             | very few... | 73             |
| 19  | 2.5% polyethylene; 5.0% 130/35° F. microwax; 25.0% 145/47° F. microwax; 67.5% 130/32° F. paraffin wax. | 640             | 33                                           | 30                                                | none...     | 76             |
| 20  | Same as 19                                                                                             | 550             | 72                                           | 30                                                | few...      | 75             |
| 21  | do                                                                                                     | 550             | 34.5                                         | 30                                                | none...     | 82             |

Examples 18, 19 and 21 clearly show an improved result where the surface tension of the coolant has been lowered to provide a difference in surface tension between the composition and the coolant of not more than 20 and particularly in the range of about 3 to 5. Examples 17 and 20 illustrate the fact that there is a greater tendency for crow's feet to form at higher speeds. Example 18 illustrates that at these high speeds a difference of surface tension of about 10 does not completely eliminate crow's feet. As stated above we preferably would employ a difference of not more than 5.

Table IV illustrates still other compositions applied at 210° F. that I have found to be benefitted by cooling in aqueous cooling baths having a surface tension lower than 60 d./cm. at 50° F.

Table IV

| Ex. | Composition                                                            | Surface tension of Composition, d./cm. at 210° F. | Viscosity Centi-stokes at 210° F. | Approximate surface tension of coolant at 50° F., above which crow's-feet appear |
|-----|------------------------------------------------------------------------|---------------------------------------------------|-----------------------------------|----------------------------------------------------------------------------------|
| 22  | 9% polyethylene; 40% 145/47° F. microwax; 61% 135/37° F. paraffin wax. | 27                                                | 24.0                              | 43 d./cm.                                                                        |
| 23  | 50% 130/32° F. paraffin wax; 50% 170/75° F. micro-wax.                 | 25.6                                              | 7.4                               | 32-35 d./cm.                                                                     |
| 24  | 2.5% polyisobutylene; 97.5% 135/37° F. paraffin wax.                   | 24.8                                              | 57                                | about 55 d./cm.                                                                  |

As previously mentioned, the lowering of surface tension of the coolant below that of water, and more particularly below 60 d./cm., at the operating temperature, becomes unnecessary when the viscosity of the coating material rises above about 100 centistokes at the application temperature. This limitation appears to apply at all speeds I have been able to obtain up to about 1000 feet per minute. When sheet speeds are not in excess of about 300 feet per minute, flow lines do not appear at any viscosity down to about 4 centistokes at temperature of application. Furthermore, there seems to be a viscosity-surface tension relationship for each speed.

I have found that any substance added to the cooling bath which will lower the surface tension sufficiently is suitable for the practice of this in-

vention. The common wetting agents such as sulfonated alcohols, amines, and esters are satisfactory. Alkyl aryl sodium sulfonates, alkylated sodium sulfo succinates, alkyl amine acetates, alkyl amines, fatty acids esters of hexitol anhydrides, alkyl dimethyl-benzyl ammonium chlorides, can be used. Alcohols such as ethyl, propyl, butyl, amyl, hexyl, septyl, octyl, nonyl, and decyl have been found advantageous to use in their normal and isomeric forms, not only alone, but also in combination with other wetting agents, where they act to suppress foam in addition to lowering the surface tension. I prefer, however, to use a wetting agent which has little tendency to foam, inasmuch as foam in the cooling bath

lowers its cooling efficiency. I have found that when foam suppressers, such as, the silicones and high molecular weight alcohols, e. g., octyl and nonyl alcohol, are used with foaming types of wetting agents good results can be obtained.

In the practice of my invention I prefer to use alcohol-water solutions, inasmuch as these solutions do not foam. In addition they are preferable since the solubility of air in such mixtures is quite low. Furthermore, alcoholic solutions can be cooled to very low temperatures without freezing or separation of the constituents.

It is to be understood that the specific examples given are intended as illustrative embodiments of the present invention and that numerous changes and modifications of the factors of the present invention are feasible which are intended

to be included within the scope of the appended claims.

I claim:

1. The process of forming on a flexible cellulosic sheet material a substantially smooth, uniform and even congealed coating substantially free of irregular flow lines which comprises applying uniformly to the sheet material a molten composition consisting essentially of a molten hydrocarbon wax having a surface tension of about 25 to about 29 dynes per centimeter at 180° F. and a viscosity not exceeding 100 centistokes at the temperature of application, and passing said coated sheet at a high speed through an aqueous cooling bath maintained at a temperature substantially below the melting point of the said molten composition, said cooling bath

containing a wetting agent, said bath having a surface tension exceeding the surface tension of the said molten coating composition by about 3 to about 20 dynes per centimeter at the moment of contact of the two.

2. The process of forming on a flexible cellulosic sheet material a substantially smooth, uniform and even congealed coating substantially free of irregular flow lines which comprises applying uniformly to the sheet material a molten coating composition comprising a molten hydrocarbon wax and a wax modifier, said compositions having a surface tension of about 20 to about 40 dynes per centimeter at the temperature of application of the coating, and passing said coated sheet at a high speed through an aqueous cooling bath maintained at a temperature substantially below the melting point of the said molten composition, said cooling bath containing a wetting agent, said bath having a surface tension exceeding the surface tension of the said molten coating composition by about 3 to about 20 dynes per centimeter at the moment of contact of the two.

3. The process of forming on a flexible cellulosic sheet material a substantially smooth, uniform and even congealed coating substantially free of irregular flow lines which comprises applying uniformly to the sheet material a molten composition having a viscosity of less than 100 centistokes at 210° F. comprising paraffin wax, microcrystalline wax, and polyethylene, and having a surface tension of about 20 to about 40 dynes per centimeter at the temperature of application of the coating and passing said coated sheet at a high speed through cooling bath maintained at a temperature substantially below the melting point of the said molten composition, said bath having a surface tension at its said temperature of from about 26 dynes to about 45 dynes per centimeter at the moment of contact of said coated sheet.

4. The process of forming on a flexible cellulosic sheet material a substantially smooth, uniform and even congealed coating substantially free of irregular flow lines which comprises applying uniformly to the sheet material a molten composition comprising a molten hydrocarbon wax having a surface tension of about 20 to about 40 dynes per centimeter at the temperature of application of the coating, and passing said coated sheet at a high speed through an aqueous cooling bath maintained at a temperature substantially below the melting point of the said molten composition, said cooling bath containing a wetting agent, said bath having a surface tension exceeding the surface tension of the said molten coating composition by about 3 to about 20 dynes per centimeter at the moment of contact of the two.

5. The process defined in claim 4 wherein the wetting agent is a monohydric alcohol.

6. The process defined in claim 4 wherein the wetting agent is isopropyl alcohol.

7. The process defined in claim 4 wherein the wetting agent is ethyl alcohol.

8. The process defined in claim 4 wherein the wetting agent is a mixture of alcohols.

9. The process defined in claim 4 wherein the wetting agent is alkyl aryl sodium sulfonate.

10. The process defined in claim 4 wherein the hydrocarbon wax is paraffin wax.

11. The process of forming on a flexible sheet material a substantially smooth, uniform and even congealed moisture-proof coating substan-

tially free of irregular flow lines which comprises applying uniformly to the sheet material a molten hot melt hydrocarbon wax moisture-proof composition having a surface tension of about 20 to about 40 dynes per centimeter and a viscosity of not more than about 100 centistokes at temperature of application, and passing said coated sheet at a high speed through a cooling bath maintained at a temperature substantially below the melting point of the said molten composition, said bath having a surface tension exceeding the surface tension of the said molten wax by not more than about 3 to 20 dynes per centimeter at the said temperature of the cooling bath.

12. The process of forming on a flexible sheet material a substantially smooth, uniform and even congealed moisture-proof coating substantially free of irregular flow lines which comprises applying uniformly to the sheet material a molten hot melt hydrocarbon wax composition having a surface tension in the range of about 20 to about 40 dynes per centimeter at temperature of application, and passing said coated sheet at a high speed through a cooling bath maintained at a temperature substantially below the melting point of said composition, said bath having a surface tension at the said temperature of the bath exceeding the surface tension of the said molten coating composition by not more than 20 dynes per centimeter.

13. The process of forming on a flexible sheet material a substantially smooth, uniform and even moisture-proof congealed coating substantially free of irregular flow lines which comprises applying uniformly to the sheet material a molten hot melt composition comprising a molten hydrocarbon wax having a viscosity of less than about 100 centistokes at temperature of application, and passing said coated sheet through an aqueous cooling bath maintained at a temperature substantially below the melting point of the said molten composition, said cooling bath containing a wetting agent, said bath having a surface tension at temperature of the bath of not more than 60 dynes per centimeter and exceeding the surface tension of the said molten coating composition at the temperature at which it contacts the bath by not more than about 20 dynes per centimeter.

14. The process of forming a continuous sheet of material coated with a moisture-proof hot melt hydrocarbon wax composition having a surface tension of about 20 to about 40 dynes per centimeter and a viscosity of not more than 100 centistokes at the temperature of application comprising coating a sheet or web of a material with said composition while molten at a speed of 300 to 1,000 feet per minute and quenching the coated material in an aqueous cooling medium which will not dissolve said composition and which has a surface tension in excess from about 3 to about 20 dynes per centimeter of the surface tension of said molten thermoplastic composition under conditions of application and not more than about 60 dynes per centimeter to form a smooth, uniform and even congealed coating on said web substantially free of irregular flow lines.

15. The process of forming a continuous sheet of material coated with a molten hydrocarbon wax composition having a viscosity of not more than 50 centistokes and a surface tension of about 20 to about 40 dynes per centimeter and comprising coating a sheet or web of a material

with said composition while molten at a speed of 300 to 1,000 feet per minute and quenching the coated material in an aqueous cooling medium which will not dissolve said composition and which has a surface tension of not more than about 45 dynes per centimeter but greater than the surface tension of said wax composition under conditions of application, to form a smooth, uniform and even congealed coating on said web substantially free of irregular flow lines.

16. In the method of coating sheets with hot melt hydrocarbon wax moisture-proof compositions having a surface tension of about 20 to about 40 dynes per centimeter wherein the coating is chilled by passing the coated sheet through a water bath maintained at a temperature to congeal said coating, the improvement comprising adding a wetting agent to said water bath in sufficient amount to lower the surface tension of the bath not exceeding by about 3 to about 20

dynes per centimeter the surface tension of said molten hydrocarbon wax at the temperature at which it contacts the water bath.

17. The improved method of claim 16 including the step of physically removing water from the coated sheet, said water containing the wetting agent picked up from the water bath, then passing the sheet through a second bath of water free of any wetting agent, and again physically removing water from said sheet.

GEORGE R. RUMBERGER.

**References Cited in the file of this patent**

UNITED STATES PATENTS

| Number       | Name    | Date          |
|--------------|---------|---------------|
| 677,320      | Norris  | June 25, 1901 |
| 1,140,873    | Carter  | May 25, 1915  |
| 2,308,638    | Balthis | Jan. 19, 1943 |
| 20 2,350,742 | Fordyce | June 6, 1944  |